

Dec. 16, 1952

L. LOVE

2,621,684

L. LOVE  
FILLING BACKED WATER RESISTANT, AIR  
PERMEABLE TEXTILE WEAVE

Filed April 6, 1950

6 Sheets-Sheet 1



Dec. 16, 1952

2,621,684

L. LOVE  
FILLING BACKED WATER RESISTANT, AIR  
PERMEABLE TEXTILE WEAVE

Filed April 6, 1950

6 Sheets-Sheet 2



INVENTOR

Louis Love

BY

*W. J. Eccleston,*

ATTORNEY

Dec. 16, 1952

L. LOVE  
FILLING BACKED WATER RESISTANT, AIR  
PERMEABLE TEXTILE WEAVE

2,621,684

Filed April 6, 1950

6 Sheets-Sheet 3



$$\Phi = 0.75 = \frac{d_3}{d_1 + d_2} = \frac{.6}{.4 + .4}$$

INVENTOR

Louis Love

*W.J. Eccleston*

ATTORNEY

Dec. 16, 1952

L. LOVE

2,621,684

FILLING BACKED WATER RESISTANT, AIR  
PERMEABLE TEXTILE WEAVE

Filed April 6, 1950

6 Sheets-Sheet 4



INVENTOR

Louis Love

BY

*H. J. Eccleston.*

ATTORNEY

Dec. 16, 1952

L. LOVE

2,621,684

FILLING BACKED WATER RESISTANT, AIR  
PERMEABLE TEXTILE WEAVE

Filed April 6, 1950

6 Sheets-Sheet 5

Fig. 1.5



INVENTOR

Louis Love

BY

H. J. Enderson

ATTORNEY

Dec. 16, 1952

L. LOVE  
FILLING BACKED WATER RESISTANT, AIR  
PERMEABLE TEXTILE WEAVE

2,621,684

Filed April 6, 1950

6 Sheets-Sheet 6



Fig. 16



Fig. 19

FACE WEAVE



Fig. 20

CHAIN DRAFT  
WOVEN FACE DOWN



Fig. 17

==BACK FILLING 11-13  
||=FACE FILLING



Fig. 21



HARNESS DRAFT

INVENTOR  
Louis Love

HARNESS DRAFT

BY

W. J. Eccleston,

ATTORNEY

## UNITED STATES PATENT OFFICE

2,621,684

FILLING BACKED WATER RESISTANT, AIR  
PERMEABLE TEXTILE WEAVE

Louis Love, Philadelphia, Pa.

Application April 6, 1950, Serial No. 154,394

12 Claims. (Cl. 139—413)

(Granted under the act of March 3, 1883, as  
amended April 30, 1928; 370 O. G. 757)

1

The invention described herein, if patented, may be manufactured and used by or for the Government for governmental purposes, without the payment to me of any royalty thereon.

This invention relates to the production of textile fabrics which are water resistant, and more particularly to composite fabrics constructed of filling backed principles, which are so designed as to effectively utilize constituent yarns of selected characteristics in constructions of near maximum cover and density within certain critical limits.

In the prior art, composite fabrics using filling backed, warp backed, double or treble principles of fabric construction have been employed for the purpose of increasing the warmth retaining qualities of cloth, and in order to secure greater weight and substance than can be obtained in a single structure which has equally fine yarns on the surface. Other known purposes of employing backed or double structures are those of appearance and a combination of appearance and weight, examples of the latter being known as reversibles, in which warp backed or double cloth structures are employed in order to provide different coloring or effects on the two sides of the cloth. These prior art constructions possess neither the principles of cloth construction which have been applied in the present invention nor do they possess the desired property of water resistance of the order or class herein disclosed by a construction within the range of critical tolerances specified, together with high thermal insulation, air permeability, shrink resistance, durability and other properties as are herein described.

One of the objects of my invention is to provide a fabric for a self-lined garment or cover, which would afford physiological comfort when worn over a wide range of climatic conditions without the need for additional protective clothing.

One of the principal factors considered in defining a fabric combining qualities which have long been sought, is the factor of superior water resistance and softness and pliability without precluding what might be termed a breathing type of fabric, which is air permeable.

A further quality of the fabric is that it affords high heat insulating properties in addition to being water resistant with a minimum of weight and maximum thickness, as compared to other textiles by which it was sought to attain qualities.

These numerous advantages and features are 55 be made to a fabric such as water resistant duck

2

obtained as a composite form in a single integrated fabric without the necessity for use of a plurality of separate independently woven fabrics each having been designed separately to have one of the advantageous qualities desired. In an effort to approximately or even remotely approach the numerous qualities above-mentioned of my integrated fabric, in accordance with prior art teaching, it was necessary to bring together the plurality of independently woven fabrics in such a relation, for example, as an outer garment (fabric) to afford the quality of water resistance, and an inner one, such as a lining to provide warmth or heat insulating properties. Of course, suitable additional means were also required, in prior art garments to secure the lining material in either permanent or detachable relation with the outer material.

So far as the inventor is aware no integrated composite fabric of a single weave has been produced in the prior art, which is like the fabric herein disclosed, relative to the critical requirements to obtain a fabric of minimum weight and maximum thickness and yet retain the qualities of water resistance and warmth in a fabric that can be practically woven by employing ordinary type yarns readily available, and by utilizing the ordinary skill and care with the usual types of machines in weaving.

As to the matter of comfort of the wearer of a water resistant article of wearing apparel, a woven fabric which has the property of air permeability, or otherwise expressed, which permits a certain amount of "breathing" action to take place to afford ventilation of the moisture vapor from wet clothing, as well as the normal skin moisture and perspiration, is far superior to a garment employing a continuous film or coating of rubber, plastic or petroleum resinous material, natural or synthetic. The continuous film, either as a coating or as a laminating film serves as a barrier to exclude water or vapor moisture, but by like token such continuous film precludes the essential property of air permeability or the "breathing" quality of the woven water resistant fabric.

As a further instance to illustrate the importance of critical factors in the choice of materials and the geometry of design and the proportioning of various factors in weaving, so as to obtain a woven fabric which is water resistant and repellent but yet air permeable and which possesses at the same time the requisite softness, pliability and draping properties, reference might

or canvas, which because of its stiffness and lack of draping qualities and lack of other desirable qualities as well, would be wholly unsuited for use as a garment of wearing apparel, except for special uses for short periods of time during which comfort is of secondary importance.

It is known that the degree of water resistance of these prior art fabrics is greatly dependent upon the fineness of their interstices, and that in the construction of these prior art fabrics, a sacrifice of softness, pliability and draping quality was made in the effort to secure a complete closure by forcing the component yarns into very close and jammed constructions.

I have discovered that the water resistance of a fabric is dependent not only upon the size of the interstices, but also upon the resilient characteristics of the material serving as a support for the water barrier, and that by providing a suitable material as a support for the water barrier in the form of an integrated backing, I have been able to obviate the necessity for the complete closure of the interstices of the facing fabric and thus permit the construction of highly water resistance fabrics which would be soft and pliable and suited for use as wearing apparel.

The present invention contemplates a composite integrated fabric structure in which the constituent yarns of selected characteristics are so arranged and proportioned within critical tolerances as to present fine interstices with fine yarns on the face of the fabric, while providing a uniformly dense cover of a resilient pile-like material on the back, the thickness of the pile-like backing being greater than that of the facing; the relative thickness of the pile-like backing being an important factor in contributing not only to the attainment of superior water resistance of the composite fabric structure but also to its economic feasibility in view of the fact that such thicker resilient pile-like backing would provide many additional desirable properties; properties, hereinafter more particularly set forth, which no other single or integrated fabric is known to possess.

The physical effect of a relatively thickly napped backing on the water resistance of a fabric whose construction details are embodied in my invention, is that it presents a thick, resilient undersurface to absorb the shock of falling raindrops on the tightly woven but still soft and pliable face fabric, thus greatly delaying breakthrough by the raindrops. It is well known that the transmission of water through a fabric is greatly increased when the undersurface is touched or rubbed. This may be explained by the capillary action of water and must be considered in the evaluation of a water resistant fabric. By providing a lofty, light, homogeneous resilient fibrous understructure, my invention prevents this capillary or wicking action by protecting the undersurface of the face fabric from being rubbed or touched.

The shrink resistance of a fabric in accordance with the present invention is aided by construction details which call for the maximum density of the component yarns. Separate linings are usually more loosely woven and have poor shrinkage properties. An integrated lining, as presented by my invention, is prevented from undesirable shrinkage by the numerous points of interlacing to the stable outer fabric, thus eliminating the distortion of a garment that would occur if a separate lining would shrink more than the outer fabric.

*Significance of air permeable, water resistant fabric having a napped pile-like backing*

There is a distinct advantage and value in providing a soft, pliable water resistant and repellent woven face of the fabric, having desirable draping qualities, in combination with the fibrous backing formed from the closely spaced, larger, soft spun, filling yarn suitably integrated and napped to provide by the open network of random raised fibers, a comparatively thick, resilient under-surface affording a continuous layer of substantially uniformly distributed, random-shaped air cells in communication with the air-permeable water resistant woven face of the fabric. A further factor contributing to the thermal insulating quality is the more stable air film and layer, entrapped between the face weave and the back filling, where it is not subject to displacement by the normal convective flow of air currents at the surface boundaries of the woven fabric. An effectively entrapped air film within a tight weave would resist displacement by convective wind velocities even though the direction of flow may exert a substantial pressure in a vector at right angles to the fabric surface, say, for example, by wind velocities of from 20 to 30 miles per hour (M. P. H.).

This uniform distribution of the layer of air cells within the fibrous brushed pile-like backing throughout the backing area of the woven facing, together with the trapped air film or layer within the weave between the back filling and the face weave, constitutes an important feature or factor contributing to the production of what may be termed a breathing type of woven, water resistant fabric, having such property independent of and apart from any special treatment by water repellent composition or method. So far as applicant knows, or has been advised, this is the first water resistant, air-permeable, woven fabric which has such desirable qualities of pliability and draping as to render it suitable for practical manufacture and use as a garment or article of wearing apparel that could be practically and economically made to specifications as to quality of yarn, control of spinning and weaving, that could be satisfactorily met, by American mills.

A further object of providing a textile having a weave, including certain physical details within prescribed critical geometric relationships as described below, is to provide a cotton face, high warp textured, Oxford weave fabric with a wool backed, napped filling, which in addition to properties of high thermal insulation, also possesses properties of shrink resistance following wetting and laundering, greater durability, and a high degree of test performance in the drop penetration test which is suitable for predicting rain resistance.

The term "greater durability" as here used is intended as a general term to embrace the concept of serviceability over an extended period of time during which the fabric is subjected to the usual wear and tear in ordinary use and service, including that of washing and laundering, after which the fabric, by recognized laundering tests has demonstrated its fitness by retaining its properties of water repellency and resistance to water and rain penetration.

While it is desirable to treat the fabric with a water repellent such as by a stearamido methyl pyridinium chloride (sold commercially and available under the trade names "Zelan" and

"Norane") tests have demonstrated and established the fact that certain of the important and characterizing features of the woven fabric, namely, those features of water repellency or resistance to rain penetration and the related resistance to drop penetration as revealed by the drop penetration test, and the draping properties and air permeability, are not dependent upon any particular water repellent treatment, durable or non-durable. Such water repellent treatments can be dispensed with, and the integrated fabric of this invention will still possess good water resistance.

In the art, the above Zelan treatment has been referred to as a "durable" type of water-repellent treatment for fabrics; it is not a permanent type of treatment. The composition and the method employed in the Zelan water repellent treatment of fabrics is understood to be set forth in the following three patents: No. 2,131,362; 2,147,392; and 2,278,417.

If desired, other types of water-repellent treatment generally recognized as being of a non-durable type, may be used. Examples of the non-durable water-repellent type are:

(a) The use of various compounds of waxes and oils of vegetable, animal or mineral origin; and

(b) The rosin-metal soap types, such as the aluminum soap type, of which there are several on the market, under various trade names.

In fabrics treated with any one of a number of the non-durable type of water-repellent agents, the water repellent action of the fabric is diminished by successive washing and laundering operations.

It is particularly important therefore that the water and rain repellent property of a fabric be present and effective by virtue of the fabric structure, resulting from the relation of the yarns, the materials, their relative sizes, and their integrated relation within critical ranges as determined by the weaving. In such a fabric, intended for use as a garment or article of wearing apparel, it is important and essential, in order to maintain these qualities of softness, and pliability of fabric which go to impart the acceptable draping properties, that in the method of weaving and in the finished woven fabric certain critical factors and constants be recognized and maintained, and that the various elements and factors involving the size, number and relation of the various yarns be substantially maintained within a specified critical tolerance range, in order to preserve those properties essential for a practicable, serviceable, and commercially acceptable product which will meet certain objective standards and recognized tests.

In carrying out the present invention, yarns of suitable characteristics are used which may be of regularly twisted cotton or spun synthetic yarns for the facing, and soft spun wool or spun synthetic yarns, alone or in combination, for the backing. If wool or any other highly shrinkable material is used exclusively, or as the major component of a blend, for the backing yarns, it is necessary in the interests of the appearance of the finished fabric that these yarns be treated to resist shrinkage. The shrinkage characteristics of wool are well known, and the use of untreated wool yarns would seriously detract from the appearance of the more stable face fabric by causing pockers after any wetting out treatment. The 75

newer synthetics, many of which are inherently shrink resistant, may be used for back filling yarns alone, or as the major component of a blend with wool or other highly shrinkable textile material, without the need for a shrink resistant treatment. The wool yarns or other highly shrinkable textile materials may be treated to resist shrinkage by any of the well known methods used in best commercial practice in either stock or yarn form.

A fabric produced according to the present invention owes its superior water resistance as well as other desirable properties to a great extent to its structural form, which comprises yarns in an arrangement which permits the attainment by a very practicable method of a facing of near maximum cover and a high overall density in addition to a thicker backing of near maximum cover. In the description of fabrics produced under the present invention, it is convenient to employ geometric constants to define the relative sizes of the yarns, their arrangement, and their properly spaced relationship to each other within certain critical limits. By means of construction details which follow in the disclosure these yarns are practicably woven into fabrics possessing high water resistance and high thermal insulation value as shown herein by results of recognized tests.

The geometric constants that have been used in my invention are delineated in the attached drawings which are provided for purposes of illustration but not necessarily for limitation. Two types of fabric and a number of modifications are shown as embodying the invention, and employing materials and factors thereof within the critical tolerances defined, to effect the essential properties in the woven fabric of water resistance and air permeability, without sacrifice of softness and pliability in obtaining draping quality and thermal insulating quality. The two types or embodiments are herein referred to as fabrics "A" and "B" and have been woven and tested.

The terms used to describe the geometric constants used in my invention are cover factor ( $K$ ), beta ( $\beta$ ), phi ( $\phi$ ), and delta ( $\Delta$ ). Subscripts 1, 2, and 3, refer to the face warp yarns, face filling yarns, and back filling yarns, respectively. "N" designates the yarn number or size. "n" refers to the number of yarns per inch.

Cover factor ( $K$ ) is defined as the ratio of the yarns per inch in the woven fabric, to the square root of the yarn size

$$\left( K = \frac{n}{\sqrt{N}} \right)$$

Maximum undistorted cover factor ( $K_m$ ) defines the point at which the perimeters of adjacent yarns are calculated to touch by assuming these yarns to be undistorted flexible cylinders.

The formulas for yarn diameters are

$$d = \frac{1}{K_m \sqrt{N}}$$

inches.

A maximum distorted cover factor ( $K_d$ ) is possible in an Oxford weave construction due to the flattening of the paired warp yarns. Both dis-

orted and undistorted values for maximum cover factors are listed below.

|                               | Numbering system | K <sub>m</sub> | K <sub>f</sub> |
|-------------------------------|------------------|----------------|----------------|
| Cotton.....                   | Inverse.....     | 28.00          | 31.40          |
| Spun synthetic staple.....    | do.....          | 28.00          | 31.40          |
| (In cotton numbering system.) |                  |                |                |
| Worsted.....                  | do.....          | 22.80          | 25.60          |
| Wool.....                     | do.....          | 15.42          | 17.28          |
| Filamentous synthetics.....   | Direct.....      | 2,300          | 2,577          |
| (In denier numbering system.) |                  |                |                |

$\beta$  (beta) is defined as the ratio of the face filling yarn diameter to the face warp diameter.

$$\beta = \frac{d_2}{d_1} = \frac{\sqrt{N_1}}{\sqrt{N_2}}$$

$\phi$  (phi) is defined as the ratio of the back filling yarn diameter to the sum of the face warp and filling yarn diameters

$$(\phi = \frac{d_3}{d_1 + d_2})$$

$\Delta$  (delta) is defined as the ratio of the back filling yarn diameter to the sum of the diameter of the face warp yarn and twice the diameter of the face filling yarns.

$$(\Delta (\text{delta}) = \frac{d_3}{d_1 + 2d_2})$$

In the drawings:

Figure 1 is a composite view showing an enlarged fragmentary broken plan of a preferred type of weave herein identified as fabric "A," having a portion of the back filling yarns cut away in order to show more clearly the high warp texture Oxford type weave of the face, and the manner in which the floated, soft spun back filling yarn is interlaced by a series of separate binder warp yarns at spaced intervals within the range of from 0.05 to .2 inch, to the Oxford weave face fabric. This enlarged fragmentary view illustrates the various warp and filling yarns of the face and the backing, yarns to scale in the approximate relative sizes determined by the constants in the formulas are within the specified range and tolerances of the critical relations and factors, which constants in this figure are  $K_1=28$ ,  $K_2=14$ ,  $\beta=1$ , and  $\phi=1$ . A repeat of the weave is shown to consist of 14 warp yarns (12 face and 2 binder) and 4 filling yarns (2 face and 2 back). A repeat of the filling yarns is indicated by arrows on the back filling yarns, #3 and #4, and on the exposed undersurface, which these yarns would cover.

Figure 2 is a draft diagram on design paper showing one repeat of weave of fabric "A" shown in Figure 1. This is a figure separate from Figure 1, but for convenience of reference and understanding, the various face warp yarns and face and back filling yarn symbols are, by appropriate arrows, keyed to and identified with the corresponding yarns in Figure 1. In Figure 2, the various face warp yarns or "ends," are numbered from 1 to 14 in the vertical columns; the separate binder warp yarns are identified as 7 and 14, and are mounted on separate harness frames. The face filling and back filling yarns are symbolically represented by the horizontal rows numbered 1 to 4 at the left of Figure 2.

Figure 3 is a chain draft or pegging plan on design paper for 10 harness frames numbered in vertical columns from 1 to 10, used in weaving the weave "A" of Figures 1 and 2. The harness frames No. 9 and 10 carry the separate system

of 2 binder warp yarns identified in Figure 2 in vertical warp columns Nos. 7 and 14. The diagram is here interpreted by the persons skilled in the art and familiar with such draft diagrams, to teach that harness frames Nos. 1, 3, 5, and 7 are simultaneously actuated to a raised position, while harness frames Nos. 2, 4, 6 and 8 are lowered, so as to interlace the face filling yarns, such as No. 2 (see Figures 1 and 2); the interlacing of face filling yarn No. 2 is more clearly shown in the upper portion of Figure 1 showing the back filling yarn removed.

Figure 4 is a drawing in and harness draft (on design paper) for 10 harness frames, and 15 reed plan for four repeats of the weave design, of fabric "A" shown in Figures 1 and 2.

Figures 1, 2, 3 and 4 are to be interpreted by reference to each other in considering the weave of weave "A," in which an independent system 20 of binder warp yarns (7 and 14 in Figure 2), are employed for interlacing the back filling yarns (3 and 4 in Figures 1 and 2). Figures 5 and 6 are other enlarged detail views of the weave of 25 weave "A," which aid in the interpretation of the draft diagrams of Figures 2, 3 and 4.

Figure 5 is a section of weave "A" taken on the line 5—5 of Figure 6 showing the face warp yarns and the tie warp yarn in section; the face filling yarn and back filling yarn are in elevation, and 30 shows the manner in which the back filling yarn is floated over twelve face warp yarns, for an extent of from 0.05 to 0.2 inch. This figure shows the various yarns in their relation to each other in a greatly enlarged but in substantially accurate 35 scaled relation.

Figure 6 is a section of Figure 5 looking in direction of the arrows and taken on line 6—6 of Figure 5, showing the face filling and back filling 40 yarns in section, and the face warp and warp tie 45 yarn in elevation. This figure shows the respective yarn sizes in substantially correct scaled relation.

Figure 7 is an enlarged diagrammatic view 45 graphically illustrating the relation between the three diameters of the yarns  $d_1$ , the face warp 50 yarn,  $d_2$  the face filling yarn, and  $d_3$  the back filling yarn. This diagram also graphically emphasizes the significance of the constant  $\phi$  (phi) equals unity in the formula

$$\phi = 1 = \frac{d_3}{d_1 + d_2}$$

Figure 8 is an enlarged fragmentary section of 55 weave "B" (shown in a plan view of Figure 17) taken generally on line 8—8 of Figure 9, showing the face warp yarns in section and the face filling and back filling yarns in elevation when the floated back filling yarn is interlaced by a pair of the face warp yarns to form a float upon fourteen 60 face warp yarns.

Figure 9 is an enlarged fragmentary section of 65 weave "B", taken on line 9—9 of Figure 8, showing the face filling and back filling yarns in section and the face warp yarns in elevation, thus showing the manner in which the face warp yarn 70 interlaces the back filling yarn at certain float intervals within a range of tolerances specified for effective napping at from 0.05 to 0.20 inch.

Figure 10 is an enlarged fragment of that portion 75 of Figure 9 showing the relation between the size and the lay of the three systems of yarn at the position of the fabric where the face warp 80 yarn interlaces the floated back filling yarn; the view serves to emphasize by graphic representation the importance of the cover factor formula

defining the constant phi ( $\phi$ ) = 0.75 (in this particular illustrative example), in terms of the size (diameters) of the three systems of yarns, as in the formula

$$\phi = \frac{d_3}{d_1 + d_2} = 0.75$$

where the symbols are as hereinbefore defined.

Figure 11 is an enlarged diagrammatic view of a modified form of a fabric herein referred to as weave "B" in which the relative sizes of the three systems of yarns in the face warp, face filling, and back filling yarns are represented substantially to scale and in accordance with the values of the constants as follows:  $K_1 = 28$ ;  $K_2 = 12$ ; beta ( $\beta$ ) = 1 and phi ( $\phi$ ) = 1. This view diagrammatically shows the undersurface with a portion of the back filling yarns removed to show the arrangement of the face warp and face filling weave, the comparative yarn diameters and the weave used to obtain this arrangement when woven face down. The numbered warp and filling yarns shown in the diagrams and drafts of Figure 14, follow the arrangement and numbers indicated in the weave "B," Figure 12. The weave draft design is conventionally constructed to show the weave to the person skilled in the art of reading and interpreting such draft diagrams. The weave of Figure 11 is identified as weave "B" to distinguish from the weave of Figure 1, identified as weave "A." Specimens of cloth were actually woven in accordance with weave "A" and "B" and tested as herein stated.

Figure 12 is a draft diagram from design paper showing one repeat of the weave "B," shown in Figure 11. This figure is separate from Figure 11, but for convenience of reference and understanding, the various face warp, and face filling or weft yarns, and back filling yarns, are, by appropriate numbers, keyed to and identified with the corresponding yarns in Figure 11. The interlacing of the various back filling yarns by the pair of adjacent warp yarns to form float lengths of from 0.05 to 0.20 inch, is indicated by the raised warp ends represented by the adjacent "X" S in blocks surrounded by the heavy band or outline.

Figure 13 is a chain draft or pegging plan for 1 repeat of the weave design shown in Figures 11 and 12, indicating to the person skilled in the art the order and sequence of operation of the 8 harness frames, identified by numeral 1 to 8 inclusive, to weave the design for one repeat, and to obtain the interlacing of the back filling yarns 3, 4, 7, 8, 11, 12, 15 and 16 (see Figures 11 and 12) by the various pairs of adjacent warp yarns on the independent harness frames.

Figure 14 is a drawing in draft design and reeding plan for one repeat of the weave design shown in Figure 11.

Figure 15 is an enlarged fragmentary view of that portion of the modified version of the fabric (weave "B") in which the face warp yarn falls below two successive filling yarns and interlaces one larger size back filling yarn. The view serves to emphasize by graphic representation the importance of the constant delta ( $\Delta$ ) in the ratio,

$$\Delta = \frac{d_3}{d_1 + 2d_2}$$

in which delta ( $\Delta$ ) defines the size of the back filling yarn in relation to the sizes of the face filling yarns. The size of the back filling yarn is important to the functional utility of a fabric produced under the present invention in which maximum density must be secured for a larger scale

70 75

backing without detracting from the density or continuity of the weave of the face fabric.

Figures 16, 17 and 18 show the weave, chain and harness draft of a modified face weave in which the face warp yarns fall below two or more successive face filling yarns to permit the incorporation of one larger size back filling yarn in a two and one arrangement with the face filling yarns.

Figure 16 shows a 3/2 twill weave repeat, 10 marked in with heavy lines carried out to a 15 warp yarn repeat in order to provide for a 15 warp yarn satin stitching arrangement for the back filling yarns (shown enclosed in the chain draft Figure 17) 15 warp ends in this case have been selected to provide a float length of from 0.05 to 0.2 inch, which may be considered suitable for effective napping.

Figure 17 is a chain draft or pegging plan of the weave of Figure 16, woven face down showing 20 the manner in which the back filling yarn is interlaced with and by the various face warp yarns.

Figure 18 is the harness draft for the face weave design of Figure 16 showing 15 harness frames for the 15 warp yarns for each repeat of the design, one harness frame being provided for each warp yarn of each repeat. The harness frames are actuated in the manner and sequence indicated in Figure 17, the chain draft or pegging plan.

Figures 16 to 18 are to be considered as a group and in their relation to each other.

Figures 19, 20 and 21 show a 15 harness satin derivative weave. The 15 harness stitching arrangement shown encircled in the chain draft of Figure 20, may be used with 2 stitching yarns instead of 1, in order to bind the backing more securely.

Figures 19, 20 and 21 are to be considered as a group and show a modified species of the weave 40 employing the various constants within the range of critical tolerance but employing a modified system of interlacing the back filling yarns to the face weave in which two face filling yarns are used for each back filling yarn. Each back filling 45 yarn is interlaced with the face filling weave by a plurality of face warp yarns at non-uniform spaced intervals within any one weave repeat, so as to form float length of the back filling of 50 variable and non-uniform length within any one repeat.

Figure 19 is a face weave design of the modified form referred to in the previous paragraph employing the chain draft or pegging plan as taught by Figure 20 to obtain the variable and non-uniform float length of any one yarn within one repeat of the weave design.

Figure 20 is the chain draft or pegging plan (woven face down) for making the face weave design of Figure 19, employing 15 warp yarns for one repeat, each warp yarn being independently actuated by a separate harness successively in combination with different harnesses during the same repeat of weave.

Figure 21 is harness draft to be considered in connection with Figures 19 and 20. There are 15 warp yarns for one repeat of the weave design, and each warp is carried on a separate harness frame.

The numbers to the left of Figure 20 and to the right of Figure 17 indicate the particular warp yarn and harness frame which is actuated to interlace the particular back filling yarn disposed in the horizontal line adjacent the particular number.

In Figures 16 to 21 inclusive the conventional symbols are employed. The "X" in a square indicates a raised warp or harness frame; on the face weave design the "X" in a square indicates a raised warp in the face of the weave, interlaced over a face filling yarn.

*Explanation of certain figures showing two "X" symbols in vertical column representing one raised binder warp yarn.*

In Figure 2, the "one repeat of the weave" of weave A, the binder warp yarns represented as warp ends or yarns 7 and 14, are each mounted on separate harness frames No. 9 and No. 10 (see Figure 3), so as to be actuated independently for interlacing with and over the back filling yarns No. 4 and 3, respectively. In Figure 2, in warp end No. 7, the "X" mark in the square opposite "No. 4 back filling" indicates that the binder warp No. 7 is in raised position and is at the surface of the weave of the cloth. The "Xa" mark in the vertical column with warp yarn No. 7, and in the horizontal row "No. 1 face filling," is consistent with the showing of Figure 1 in which the face filling yarn No. 1 is below the back filling yarn No. 4 which, in turn, is below and interlaced by binder warp yarn No. 7. (See Figure 1 and Figure 2.) The second and upper "Xa" symbol in the vertical row of binder warp No. 7 (see Figure 2), does not mean or symbolize a relation in which the No. 1 face filling yarn is in contact with or directly interlaced by the raised binder warp No. 7, which is in raised position (see Figure 2), on the harness frame No. 9 (see Figure 3) above the face filling yarn No. 1 as indicated by the symbol "Xa" in vertical warp column No. 7. The back filling yarn 4 is directly interlaced by binder warp yarn 7; said back filling 4, is also above the face filling yarn 1, and is directly interposed between the binder yarn 7 and the face filling yarn 1.

The explanation in the previous paragraph, directed to an understanding and interpretation of these portions of the diagrams of the drafts on design paper showing one repeat of the weave, and chain draft, at those warp yarns which interlace with and tie in the back filling yarns 3, 4 which also covers a face filling yarn, is equally applicable to other figures such as Figures 11, 12, 16, 17, 19 and 20 in which, more than one "X" symbol appears in a vertical column representing any one warp yarn, which at a certain time during one repeat, is raised to a position to interlace with, and tie-in the back filler yarn, with the face warp yarns. It is not thought to be necessary to repeat the explanation of a fairly comparable situation which may exist in the other figures such as Figures 11, 12, 13, 16, 17, 19, and 20. The unfilled or blank squares, in horizontal rows in one repeat of weave, and harness draft diagrams, usually represent the filling yarn floated at the face or surface of the weave of the textile, with the warp yarn in interlaced relation below and under said filling yarn; this applies to the diagram of a draft design of one repeat of the weave, or harness draft of the common weave. The weave of the present textile is not the conventional simple weave but includes a back filling yarn floated on the back of a facing weave, which in turn includes a separate and independent system of face filling yarns (such as 3, 4 of Figures 1 and 2). The usual simple type of draft design diagram to show the conventional common weave cannot be used alone, but addi-

tional means must be provided to identify the back filling yarn, and indicate its relation to the other yarns, and to distinguish from the face filling yarn; it is essential also to indicate the manner and means employed for integrating the back filling yarn into the weave of the fabric to enhance the water resisting characteristics of the face weave. The conventional type of draft design diagrams have herein been modified sufficiently by appropriate symbols to clarify the disclosure.

In the absence of an enlarged view substantially to scale, for each of the modified forms, to show the weave and lay of each of the yarns, in the woven fabric, such as shown in Figures 1 and 11, the draft design diagrams of one repeat of the weave and harness draft will convey to the person skilled in the art sufficient information to enable him to set up the harness reed and heddle mechanism of the loom to weave the cloth in accordance with the manipulation of the harness and chain draft diagrams for one repeat of the weave design for the various modified forms hereinafter shown (see Figures 16 to 21).

Referring in greater detail to the drawings, Figure 1 is a composite view of the undersurface with a portion of the back filling yarns cut away showing the high texture warp yarns in the preferred type of fabric using the oxford weave for the face. In single fabrics of high warp textures, the oxford weave lends itself to the attainment of high overall densities essential to the water resistance of a fabric. In the present high warp textured fabric with an additional floated back filling of a defined size larger than the face filling, high overall density for the face of the fabric is best obtained with an oxford weave by employing a separate system of binder yarns. While various means and methods may be employed for effecting the uniform interlacing and integration of the back filling to and with the woven face, Figures 2, 3, and 4 showing the weave, chain and harness draft for one repeat of the weave, when properly understood and interpreted by the weaver skilled in and familiar with his art, is sufficient to indicate the sequence of manipulation of the warp and binder yarns to effect the particular form or method of uniform integration.

Figure 5 is a cross-sectional view of the warp 50 yarns taken on the lines and looking in the direction of the arrows 5-5 of Figure 6, showing the position of the binder warp yarns (b). At 6-6 the binder warp yarn b is above the face filling, but remains hidden under the paired warp 55 yarns W, thus presenting an unbroken oxford face weave effect. The adjacent binder yarns b are below the back filling yarns and show the manner in which the back filling yarn is floated for 12 face warp yarns. These adjacent binder 60 yarns alternate weaving above and below successive face and back filling yarns as shown by the dotted lines in Figure 6.

Figure 6 is a cross-sectional view of the filling 65 yarns, taken on the line and looking in the direction of the arrows at section 6-6 in Figure 5.

These Figures 5 and 6 show the various yarns in their relation to each other in greatly enlarged, but in substantially accurate scale. The warp cover factor  $K_1=31.4$  and represents a constant, which when multiplied by the square root of the cotton yarn size or number, indicates the number of cotton yarns per inch to be used in order to obtain the flattened effect of the paired warp 70 yarns. A fabric using a 36/2s cotton warp yarn

## 13

with a cover factor of 31.4 would have approximately 133 yarns per inch

$$(31.4 \times \sqrt{\frac{36}{2}} \text{ or } 18)$$

A float of 12 threads of this number would therefore occupy a length of .0903 inch

$$\left( \frac{12}{133} \text{ inches} \right)$$

which falls within the prescribed limits of .05 to .2 inch—the specified range of float lengths desired for effecting napping.

Figure 6 also shows the yarn sizes in substantially correct scaled relation. The paired face warp yarns ( $w$ ) may be observed to do most of the bending and weave with the face filling yarns ( $F$ ) in a one up and one down arrangement, known as the oxford weave. It is shown that one-half of the perimeter of the contiguous face filling yarn  $F$  is interlaced by the face warp yarn ( $w$ ). This relationship between the diameters of warp and filling yarns is supplied by the ratio  $\beta$  (beta) and for this example is shown to be 1 (one-unity), since the diameters of these yarns are equal.

The geometric principles used for the face oxford weave fabric to increase its water resistance require the maximum number of face filling yarns ( $n_2$ ) that can be obtained with a given  $\beta$  (beta). The formula for approximating this maximum number per inch of the cloth in the inverse yarn numbering system is:

$$n_2 (\text{max.}) = \frac{K_m \beta \sqrt{N_2}}{1 + \beta}$$

in which

$$\frac{K_m \beta}{1 + \beta}$$

equals the filling cover factor ( $k_2$ ), and the desired  $\beta$  approximates 1.2. In Figure 6,  $\beta$  is shown to be 1.0.  $K_m$  is given for cotton at 28, and by substitution, the resultant filling cover factor ( $K_2$ ) = 14, which is a constant, when multiplied by the square root of the cotton filling yarn size, results in a close approximation of the maximum number of filling threads that can be placed in a fabric of maximum warp texture.

Certain of these principles are known in the art and have hitherto been applied only to single cotton fabrics for the improvement of their water resistance, but such cloth was not successful as lacking pliability and draping quality and other disadvantages as herein noted.

In order to obtain a fabric having superior and outstanding water resistance, my invention provides for an additional system of closely spaced, larger, soft spun, back filling yarns suitably floated, and integrated and napped as a backing. Figures 1-6 have been presented to illustrate the relative positions, the relative sizes, and the spatial requirements of the various yarns used, and to designate the method of their integration into a stable, practical fabric. The following explanation and formulas are provided in order to present the means of reducing the scale of illustrated diagrams to the scale of a fabric in terms of yarn sizes, through the employment of constants ( $K$ ) which express the relationship between construction variables such as yarns per inch ( $n$ ) to the yarn size or number ( $N$ ), and ratios  $\beta$  (beta),  $\phi$  (phi), and  $\Delta$  (delta), which define the relative sizes of the yarns used.

It may be seen in Figures 5 and 6 that the di-

## 14

ameter ( $d_3$ ) of the back filling yarn may be larger than the diameter ( $d_2$ ) of the face filling yarn since the back filling yarns do not interlace as frequently with the face warp yarn. The size of the back filling yarn that may be used is provided for by the ratio  $\phi$  (phi) = 1 in the formula

$$\phi = \frac{d_3}{d_1 + d_2}$$

which, interpreted, means that the diameter of the back filling yarn ( $d_3$ ) is equal to the sum of the diameters of the face warp yarn ( $d_1$ ) and the face filling yarn ( $d_2$ ). This relation is shown in Figure 1 in which the back filling yarn is shown to scale as being of a diameter equal to the sum of the diameters of the face warp and filling yarns respectively. Figure 7 is an enlarged diagrammatic view graphically illustrating the relation between the three diameters of the yarns, the face warp yarn ( $d_1$ ), the face filling yarn ( $d_2$ ), and the back filling yarn ( $d_3$ ) where  $(d_1) = d_2$  and where

$$\text{beta } (\beta) = 1 = \frac{d_2}{d_1}$$

This diagram also graphically emphasizes the significance of the constant  $\phi$  (phi) equaling unity in the formula

$$\phi = 1 = \frac{d_3}{d_1 + d_2}$$

With the number of warp yarns that have been prescribed for the single fabric ( $K_1 = K_1 \sqrt{N}$ ), the face filling and added back filling are woven alternately in a 1 and 1 arrangement, or in the 2 and 2 arrangement as shown in Figure 2.

The number of face filling yarns per inch that should be used in an equal arrangement with the back filling yarns (1 and 1, or 2 and 2) may be defined as the maximum obtainable in the weaving of the integrated structure within certain calculated tolerances. This definition allows for a reduction from the number prescribed for a single fabric, which number cannot be reached due to the jamming of the larger back filling yarns.

Since greater thickness, compactness, and a more uniform distribution of the fibrous understructure are obtained through the employment of larger back filling threads as prescribed by phi ( $\phi$ ) = 1, in the ratio

$$\frac{d_3}{d_1 + d_2}$$

and since these factors contribute greatly to the attainment of superior water resistance as well as higher thermal insulation, the relatively larger size of the back filling yarns is used, while a reduction of the face filling yarns per inch is permitted within defined limits to allow for the spatial requirements of the larger back filling yarns and their integration into the fabric structure. The preferred range of values for phi ( $\phi$ ) is .9 to 1.2, while a permissible range is .7 to 1.3. The consequent reduction of face filling yarns per inch caused by the spatial requirements of the larger back filling yarns when phi ( $\phi$ ) is greater than 1, is considered in the modified formula for  $n_2$  (maximum)—

$$n_2 (\text{max.}) = \frac{K_m \beta \sqrt{N_2}}{(\phi)(1 + \beta)}$$

when phi ( $\phi$ ) > 1.0. While other means, herein disclosed, may be used to attach the larger, soft spun, back filling yarns to the face fabric, the

employment of binder yarns solely for this purpose is preferred because these yarns permit a more closely integrated structure of the component yarns within the prescribed relationships which provide for superior water resistance. The binder yarns (b) may be placed between the paired face warp yarns (W,W) of the oxford weave at specified intervals, so that a repeat of the interlacing of these binder yarns (b) with the soft spun back filling yarns (BF) permits a float of the back filling yarns of a length of from 0.05 to 0.20 inch, within the range of tolerances for effective napping. These binder yarns (b) may weave with the face filling yarns along with the paired warp yarns (W,W), except that they alone engage the back filling in a specified arrangement, one of which is shown by enclosed Xs in the weave of Figure 2. These binder yarns (b) are assigned to fall beneath the paired warp yarns (W, W) and leave the appearance of the face unchanged. The binder warp yarns may have a smaller diameter than the regular face warp yarns and may be of a different material such as nylon.

Since the float length of the soft spun, back filling yarns is important to the effective napping properties of these yarns, the definition of this length, in inches, makes it independent of the scale of the fabric. The float length defined in inches permits the calculation of the number of warp yarns between interlacing points after the determination of the number of warp yarns per inch, the formula for which is  $n_1 = K \sqrt{N}$ .  $n_1 \times$  float length (inches) = member of yarns between interlacings. A minor adjustment in the number of warp yarns between interlacing points may be necessary in order to provide suitable stitching points for the binding yarns so that they do not disturb the appearance of the face fabric. The defined float length range of .05 to 0.2 inch permits an adequate latitude for the utilization of various types and qualities of fibers which may be used in the back filling yarns for the attainment of a desirable lofty, light, durable fibrous understructure through napping.

Figure 3 is a harness draft showing one repeat of the design of the fabric weave shown in Figures 1 and 2. An X mark within the squares represents a raised warp yarn lying over the face filling yarn. A ten harness draft is shown. The raised binder warp yarns are shown as an X within a square, in the columns indicated by the arrows in Figure 2. This draft indicates the floating of the back filling yarn (BF) over 12 warp yarns (W) before such back filling yarn is tied to the face by the binder warp yarn (b) which is carried on a separate harness 9, 10 (Figure 3) from the face warp yarns (Figure 3, yarns 1 to 8 inclusive). For one repeat of the fabric design, there are two tie warp yarns, each carried on separate harness frames. The relation of the back and face filling yarns to the face warp and the warp yarns respectively is indicated in Figure 2 by the identifying designations 1, 2 face filling and 3, 4 back filling, in the column to the left of the draft. In the draft weave one repeat diagram (Figure 2), each vertical row of squares represents one warp end of yarn, and each horizontal row of squares, represents a filling-weft-yarn, also referred to as a "pick" of the weave. In Figure 3, the "chain draft 10 harness" diagram, the vertical numbered rows represent a harness frame, and not merely one warp yarn as in Figure 2.

In the conventional draft design diagrams of a common weave, for either the harness or the chain (or pegging plan) draft, or plain weave design, the squares which are filled in or, with some identifying symbol, represent a raised harness, and a warp yarn in a correspondingly raised position in the "shedding" of the filling or weft yarn. In the diagram of one repeat of the weave design, a square filled-in with a symbol such as an "X," or other symbol, represents a raised warp yarn, usually at the face or surface, and disposed above and interlaced with a filling yarn.

A chain draft or pegging plan on design paper indicates how and in what order the harnesses must be lifted so that the warp ends drawn through them will interlace with the filling according to the desired weave; in other words, the chain draft or pegging plan shows which harnesses are to be raised and which lowered on each pick.

Figure 11 is a composite view showing an enlarged fragmentary broken plan of a modified version of a highly water resistant fabric, having high thermal insulation value herein identified as weave "B." A portion of the back filling threads is cut away in order to show the high warp texture Oxford type weave of the face, and the manner in which the floated, soft spun, back filling yarns are interlaced, by raising the paired

face warp yarns above them in a uniformly distributed arrangement which permits the back filling yarns to float over the warp yarns for lengths which have been defined as within the range of from 0.05 to 0.20 inch. The float length being important to the effective napping properties of the back filling yarns is defined in inches, independent of the scale of the fabric. The float length determines the number of warp yarns between interlacing points of the back filling

yarns and is used to determine the weave and the number of harness to be used. The stitching arrangement with the paired warp yarns is shown enclosed in weave B of Figure 12 and illustrated in Figure 11. The vertical spaces in the weave B, numbered from 1 to 16 represent the warp yarns and are attached by lines to the corresponding yarns in the diagram. A repeat of 16 warp yarns would ordinarily necessitate the requirement of 16 harness for the weaving of this fabric, but in this case the paired warp yarns, in an Oxford weave arrangement, weave as one yarn and may be placed on eight harnesses as shown by the drawing in plan in Figure 14 and chain draft in Figure 13. The stitching ar-

range with the paired warp yarns has been therefore based on an eight harness satin weave which permits a uniform distribution of stitches throughout the fabric. The selection of a stitching weave with uniform distribution of stitching points is a precaution taken to prevent a distortion that could occur in a fabric, especially after being subjected to laundering. This system of stitching may be modified by other weaves using more or less harnesses in order to provide de-

sired float lengths, uniformly spaced. Figures 12 to 14 have been provided to show the method of integrating the back filling yarns, which indicate to the persons skilled in the weaving art, the order and sequence in which the yarns for the face warp, face filling, and back filling are manipulated by the harness, reeding plan, and the shuttle arrangement for the face and back filling yarns respectively.

The constants which define the numbers and relative sizes of yarns in a fabric using this warp

stitched method of integrating the back filling yarns may be determined by formulae which have been presented for the binder stitched fabric "A." In Figure 11,  $K_1=28$ ,  $K_2=12$ ,  $\beta=1$ , and  $\phi=1$ . These constants differ from those of the preferred weave "A" in that  $K_2$  in Figure 1 equals 14. This difference in the filling cover factors is illustrated by the comparative closeness of the back filling yarns in Figure 1 and the closeness in Figure 11. The filling cover factor  $K_2=14$  in Figure 1 defines the maximum cover or closeness of the yarns from the formula:

$$K_2 = \frac{K_m \beta}{1+\beta} = \frac{28 \times 1}{1+1} = 14$$

The filling cover factor ( $K_2$ ) of 14 cannot be obtained in weave "B" of Figure 11, while retaining the other constants in view of the spatial requirements of the interlacing paired warp yarns. These yarns are part of the face fabric and are firmly bound. They therefore are more restricted than separate binder warp yarns which may be of a smaller diameter and more pliable. Greater cover for the backing yarns under these conditions may be obtained through the use of binder yarns. The employment of binder warp yarns is therefore preferred because they permit a more closely integrated and compact fabric structure of the component yarns as defined. Weave "A" using binder yarns is shown to have a higher degree of water resistance by the results of recognized test methods used to evaluate this property. These results are presented and follow in this disclosure.

Since the physical effect of a soft spun, larger, back filling yarn, integrated in the prescribed manner, improves the water resistance of a fabric to the extent that this property is not entirely dependent on the rigid adherence to the openness or tightness as presented by the prescribed formulas, more open structures which to a great extent retain the superior water resistance and other properties as claimed, may be permitted within defined cover factor limits and weaves. These relaxed restrictions permitted with my invention are important as a factor contributing to pliability, and draping property of a more open fabric without seriously impairing its inherent water resistance. Fabric "B" with approximately 20% less than the maximum tightness as determined by formula, is shown by recognized tests to have a water resistance far superior to a single fabric without the integrated floated backing as herein disclosed.

The significance of  $K_1$  and  $K_2$  in the description of my invention is that the values for these constants provide a convenient method of indicating the cover in projection of each of two systems of yarns (warp and filling) in terms of the construction variables ordinarily used, such as textures and yarn sizes. This cover  $c_1$  may be expressed in percentage by the formula:

$$\frac{K_1 \times 100}{K_m} = \frac{d \times 100}{p} = c_1 (\%)$$

A cover factor of 28, from the above formula, indicates 100% cover. It may be seen in Figures 1 and 11 that the proportion of the area covered by the projection of the warp yarns which have a cover factor of 28 is 100%. It may also be seen that the proportion of the area covered by the projection of the filling yarns is limited to 50%, due to the space required for the interlacing of the warp yarns. This space is occupied by the distance equal to the diameter of the warp

yarn, which is equal to the diameter of the filling yarn ( $\beta$  (beta)=1). Fifty per cent cover is expressed by the cover factor

$$K_2 = \frac{K_m \beta}{1+\beta} = \frac{28 \times 1}{1+1} = 14$$

A reduction in the warp cover as expressed by the warp cover factor ( $K_1$ ) allows a corresponding increase in the filling cover as expressed by the filling cover factor ( $K_2$ ), by the space made available for the bending of the filling yarns.

Total cloth cover (C) is only possible when one system of yarns such as the warp yarns in Figures 1 and 11 have a maximum cover factor (K=28). Systems of yarns (warp, filling) having more than a cover factor of 14, restrict the opposing system from making a complete closure due to the insufficient space allowed for the bending of the opposing system. Cloth cover (C) may be defined by the formula:

$$C = \frac{1 - (K_m - K_1) \cdot (K_m - K_2)}{K_m^2} \times 100 (\%)$$

The principles used to obtain a greater measure of water resistance in a single fabric necessitate maximum warp cover within very close tolerances and maximum tightness or compactness for the filling yarns. The critical nature of these requirements to the water resistance of a single fabric is indicated by the high quality, uniform, multi-ply yarns, spun and woven under carefully controlled conditions. It is evident that the need of high warp texture to provide complete closure is to a large extent overcome by the added support, supplied by an extra system of soft spun filling yarns of maximum cover and thickness. The softness of these back filling yarns, which is an added aspect, enables them to flatten and fill the interstices. While in the prior art single fabric high warp cover is the sole means of obtaining maximum cloth cover; in the wool backed fabric here disclosed, it is only a supplementary means or a part one of numerous elements in a successful whole. The greater cover and uniform density thus obtained with the soft spun filling yarns permits a reduction of the high warp textures within defined limits without seriously impairing the water resistance of the integrated structure.

Filling cover factor limits have been defined as those imposed by practicality, viz., the maximum filling yarns obtainable in the integrated structure. This definition allows for a reduction from the calculated cover factor which, at best, can only be a close approximation due to the irregular nature of the cloth structure, and the ability of the weaving mechanisms to process the varied constructions. Preferred weave "A" is shown to have a filling cover factor of approximately 20% less than the prescribed values for filling cover factor  $K_2$  and yet possess superior water resistance. A further extension of  $K_2$  tolerances to include the use of larger values for  $\phi$  must be considered. Within the specified critical tolerances, water resistance much superior to that of an equivalent single fabric is made possible by a combination of factors, such as the high warp texture, the physical effect of a large soft spun backing, and method of integration.

The openness of a fabric, which to a large degree affects the water resistance of the integrated structure, can be determined from the cover factors of the various yarns used. The limits of openness, however, are governed by practical considerations in fabric manufacture. The pre-

scribed fabric calls for one system of yarns, such as the warp yarns, to do all the bending or crimping so as to permit the proper integration of an additional system of large backing yarns. Such a system requires a very high cover factor. A reduction in the value of this warp cover factor would permit an increase in the value of the cover factor for the filling yarns. The space remaining between the reduced number of warp yarns per inch by using a lower warp cover factor would permit the bending and consequent increase in the number of filling yarns per inch.

This investigation brought out that practical fabrics incorporating my invention could be made within certain specified tolerances and yet retain a large measure of effective water resistance. These tolerances or limits of openness may be expressed as a percentage of the prescribed cover factors for these fabrics as follows:

$$K_1 = K_f(1 \pm .30)$$

$$K_2 = \frac{K_m \beta}{\phi(1 + \beta)} (1 \pm .35)$$

Although it is preferred that

$$\beta \text{ (beta)} \frac{d_2}{d_1}$$

have a value approximating 1.2, the geometric principles that have been used with my invention may be modified to include a range of values for  $\beta$  of .9 to 1.3, and an extended range of permissible values for  $\beta$  of .75 to 1.5. Similarly, these geometric principles may be modified to include a range of values for

$$\phi \text{ (phi)} \frac{d_3}{d_1 + d_2}$$

of .9 to 1.2, and an extended range of permissible values for  $\phi$  of .7 to 1.3.

The geometric principle calling for a high warp texture with an Oxford weave of a textile fabric may be used in the practice of my invention to include other short float weaves for the face fabric such as twills, satins, or their derivatives, having warp yarn floats of up to four face filling yarns and filling yarn floats of up to eight warp yarns. The greater float of eight warp yarns may be used because the higher warp texture results in shorter float lengths. In addition, the float of eight warp yarns admits the possibility of using two warp yarns as one. These modifications may exist within the geometrical constants and tolerances which have been set up to described the fabrics of my invention in both the preferred binder stitched type "A" and the modified warp stitched type "B."

Certain other modified forms are herein shown (see Figures 15 to 21), wherein the face fabric weaves include a weave in which the warp yarns fall below two or more successive face filling yarns in the weave repeat with an arrangement of two face filling yarns to one back filling yarn. The size of the back filling yarn using this arrangement may be determined by the ratio  $\Delta$  (delta) which is a constant similar to  $\phi$  (phi).  $\Delta$  (delta) is defined as the ratio of the back filling diameter to the sum of the warp diameter and twice the diameters of the face filling yarns

$$\frac{d_2}{d_1 + 2d_2} = \Delta$$

In the description of this modified version, utilizing two face filling yarns to one back filling yarn,  $\Delta$  (delta) replaces  $\phi$  (phi) in defining the size of the back filling yarns, while the other

constants such as  $K_1$ ,  $K_2$ , and  $\beta$  (beta) are retained to define the geometry of the face fabric. The limits of yarn floats defined in the modification of the face fabric weaves to other than

5 the Oxford weave are also retained. These permit the use of short float weaves, having warp yarn floats of up to four face filling yarns by the warp yarns and filling floats of up to eight warp yarns. The desired value for  $\Delta$  (delta) with the two face and one back filling yarn arrangement is .9. A preferred range of values is from .8 to 1.2, and a permissible range is from .6 to 1.3. With this modification, binder stitching or warp stitching may be employed.

10 15 Figure No. 16 is a conventional draft design diagram of the face weave of a modified form employing two face filling yarns to one back filling yarn, and shows a

20  $\frac{3}{2}$

25 twill weave carried out to a 15 warp yarn repeat in order to provide for a 15 warp yarn satin stitching arrangement for the back filling yarns

30 35 (shown by heavy boxed square in the chain draft diagram for weaving face down, in Figure 17). With this system of stitching the back filling to the woven face, a float of 15 face warp ends has been indicated which would provide a float length of the back filling yarns approximating the length of the back filling yarns of the preferred weave "A," provided the warp cover factors ( $K_1$ ) and warp yarn diameters ( $d_1$ ) are equivalent.

35 Figure No. 17 is a conventional representation by diagram of a chain draft-woven face down of the draft diagram of the face weave shown in Figure 16.

40 Figure No. 18 shows a harness draft diagram for making the textile design shown in Figures

45 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 95

face of the fabric. Such fibers form a layer of relatively low density (as compared with the relatively tightly woven face) which serves to entrap intercommunicating air cells in a layer of greater thickness than the film of air within the weave entrapped between the face weave and the back filling yarn. The entrapped air cells within the napped fibers or back of the back filling yarn are uniformly distributed over the back face of the back filling yarn and in such position may carry off and ventilate body moisture vapors such as from perspiration. The high vapor pressures incident to the conditions of body temperature and higher relative humidity are factors which contribute toward the elimination of body perspiration through the type of "breathing" fabric disclosed herein, but yet will exclude and prevent the penetration of water moisture when the woven face of the fabric is on the outside of any garment where it is exposed to the weather elements.

In accordance with the prescribed principles and physical details, two wool backed fabrics, samples "A" and "B" have been constructed (fabric "A" being representative of my invention, employing binder yarns and fabric "B" being warp stitched). These fabrics have been tested and are shown to possess an outstanding degree of water resistance in addition to high thermal insulation value, excellent launderability, and increased durability. They use regular commercial 2-ply cotton yarns and at their maximum texture maintain a soft pliability. The wool yarn for the back filling was previously subjected to a shrink resistant treatment. The water resistance of these fabrics was found to exceed that of the best American version of the English Shirley cloth, even after prolonged laundering.

Fabric "A" of these test fabrics had  $K_1$  about 33.54,  $\beta$  about 1.225,  $\phi$  about 1.07, and  $K_2$  about 11.25.

These two fabrics may be generally described as woven fabrics of high water resistance, having unnapped face material of a short float weave, having warp yarn floats of up to four face filling yarns and face filling floats of up to eight face filling yarns, the face yarns being integrated with additional floated filling as a napped backing. The ratio of the count (number per inch) of the face filling yarns to the count of the back filling yarns is a constant  $Z$  which in fabric "A" is the integer 1, and in fabric "B" is the integer 2. The cover factor in both types of fabrics is represented by the formula

$$K_1 = \frac{\text{Number of warp yarns per inch}}{\sqrt{\text{warp yarn number}}} = 31.4(1.0 \pm .35)$$

The ratio between the diameters and the face filling yarns and face warp yarns is represented by the constant  $\beta$  in the equation

$$\beta = \frac{d_2}{d_1}$$

said  $\beta$  having a value of .1 to 1.3. The ratio between the diameters of the face warp, face filling and back filling yarns in both fabrics is represented by  $X$  in the formula

$$X = \frac{d_3}{d_1 + d_2 Z}$$

in which

$d_3$  = diameter of the back filling yarn  
 $d_2$  = diameter of the face filling yarn  
 $d_1$  = diameter of the face warp yarn.

said  $X$  having a value of .7 to 1.3 when  $Z=1$  and a value of from .6 to 1.3 when  $Z=2$ . The cover factor of the face filling yarns in both fabrics is represented by the formula

$$K_2 = \frac{\text{Number of face filling yarns per inch}}{\sqrt{\text{Filling yarn number}}} = \frac{28\beta(1.0 + .35)}{X(1 + \beta)}$$

wherein  $\beta$  and  $X$  have the above meanings. It will be seen that these values exactly correspond to those given in the earlier set forth cover factor formulae employing  $\phi$  and  $\Delta$  values, respectively.

The tests of the various properties possessed by the wool backed and control cloth were performed in accordance with Federal Specification for Textiles, General Specifications, Test Methods, CCC-T-191a, dated April 23, 1937, and supplement dated October 8, 1945, with the following results:

According to the drop penetration test, wool backed fabric, weave "A" resisted water penetration for over 72 hours; and weave "B" resisted water penetration for over 14½ hours, whereas a single cotton Oxford water resistant fabric, which represents the best American commercial version of the English Shirley cloth, and which was treated identically the same as the wool backed fabrics with a water repellent compound, resisted water penetration for approximately 54 minutes. Weave "A" of the present invention was tested by the drop penetration tester in the greige, without finishing, napping, or a water repellent treatment, desized, and was shown to resist water penetration for over 31 hours.

The durability of the water resistance of the wool backed fabrics, type "A" and type "B," as compared to the single cotton Oxford water resistant fabric, was shown by the results of the drop penetration tests after these fabrics were given a prescribed laundering and wet mechanical action treatment. After this treatment, the wool backed fabric, type "A," resisted water penetration for an average of over 20 hours, type "B," for over 2 hours, and the cotton Oxford, single, water resistant cloth, for under 16 minutes.

The thermal insulation values of the wool backed fabrics, were compared to that of a combination of a single cotton Oxford fabric and a regular standard all wool Army lining cloth of approximately the same weight as the wool backing of the wool backed cloths. The values obtained for the wool backed cloths showed that these cloths had approximately three times the thermal insulation value of the separate cotton and wool lining material tested together.

The shrinkage results of the wool backed fabrics, after being given a regular cotton laundering, showed that the shrinkage of type "A" was 4% warpwise by 0% fillingwise, and that the shrinkage of type "B" was 5% warpwise by 0% fillingwise. These results are considered acceptable by the Army, for whom woolen fabrics must not shrink more than 5% warpwise by 4% fillingwise, after a much less severe wool laundering. The differences in the shrinkage characteristics between cotton and woolen fabrics would be evidenced in the distortion that could occur in a cotton, wool lined garment after laundering; a laundering problem which has been overcome by means of the integrated lining as prescribed by the present invention.

The tear resistance, which is very poor especially across the low number of filling yarns

of a single cotton Oxford water resistant fabric, has been improved by over 100% by the addition of an extra system of wool filling yarns. The integrated wool lining, in turn, is much more durable than a separate wool lining due to the added support provided by the more durable face fabric.

The preceding test results together with evaluations have been presented on properties that are measurable by recognized laboratory test methods. Other properties, less measurable, but evident are appearance and comfort. Versatility and economy may also be mentioned.

A separate thin cotton fabric of the weight used for the face fabric of my invention has poor crease resistance. Combined with a resilient backing, as prescribed in my invention, a thicker, more resilient fabric is formed which prevents the sharp bending which causes creases. A garment made of the backed fabric thus retains its shape longer and greatly enhances the appearance of the wearer.

A garment made of the backed fabric is less binding than that requiring a separate lining or sweater. The firmly bound napped backing material does not have the restricting and creeping action of a loosely held, seamed, lining material, especially in the arms and armpits. The greater resiliency of the backed fabric prevents it from clinging to the body.

This cloth as defined has useful application for many supplementary items of apparel and equipage. Steps have been taken to use it in gloves, hats, coats, raincoats, snow suits, trousers, bed rolls, ground cloths. It may be used for tarpaulins, foot coverings, tents, shoe lining, filter cloths, and auto tops (without napping).

The practicality of the backed cloth from the standpoint of production and economy may be shown by the following estimates. The question of costs and price, of course, is one involving a number of relative factors. While no costs for the backed fabric on a production scale are available, it may be reasonably and logically estimated from costs of sample yardage that it will be roughly \$2.60 per square yard for a 16 ounce fabric. In comparison the cost of a separate cotton fabric of a fairly comparable construction to the facing is approximately \$1.30 per square yard. A separate wool or spun nylon lining which may be used with this material to give a comparable measure of thermal insulation would have to be at least 12 oz. per square yard and cost approximately \$2.80. Thus, a combination of materials of expected equivalency in thermal insulation but which would have inferior water resistance and other less desirable properties as described, would cost approximately 58% more and use up 50% more wool or spun nylon, meanwhile adding unnecessary weight. To these savings must be added those of the costs in fabricating separate linings into a garment of comparative thermal insulation. In addition, wool and nylon materials are so difficult of procurement during periods of emergency that these materials are placed on the critical conservation of material list by the Army.

What I claim:

1. A woven fabric of high water resistance, having a face material of a short float weave, said weave having warp yarn floats of up to four face filling yarns and face filling floats of up to eight face warp yarns, said face yarns being integrated with additional floated filling as a backing, said fabric comprising face warp and filling

yarns, and back filling yarns floated under said woven face to provide a back surface, in which the ratio of the number of said face filling yarns to the number of said back filling yarns is an integer of from 1 to 2, in which the diameter of said back filling yarns substantially exceeds the diameter of said face yarns, and in which the face warp has a cover factor whose value substantially exceeds the value for the cover factor of the face filling.

2. A water resistant fabric according to claim 1, wherein said face warp yarns and face filling yarns are members of the group consisting of cotton and spun synthetic staple yarns, and wherein said back filling yarns are members of the group consisting of wool and spun synthetic staple yarns.

3. A water resistant fabric according to claim 1, wherein said face warp and face filling yarns are cotton and wherein said back filling yarns are shrink resistant wool.

4. A woven fabric of high water resistance, having an unnapped face material of a short float weave, said weave having warp yarn floats of up to four face filling yarns and face filling floats of up to eight face warp yarns, said face yarns being integrated with additional floated filling adapted to form a napped backing, said fabric comprising face warp and filling yarns, and back filling yarns floated under said woven face adapted to provide a pile-like back surface, in which the ratio of the number of said face filling yarns to the number of said back filling yarns is an integer of from 1 to 2, in which the diameter of said back filling yarns substantially exceeds the diameter of said face yarns, and in which the face warp has a cover factor whose value substantially exceeds the value for the cover factor of the face filling.

5. A woven fabric of high water resistance, having an unnapped face material of a short float weave, said weave having warp yarn floats of up to four face filling yarns and face filling floats of up to eight face warp yarns, said face yarns being integrated with additional floated filling adapted to form a napped backing, said fabric comprising face warp and filling yarns, and back filling yarns floated under said woven face adapted to provide a pile-like back surface, in which the diameter of said back filling yarns substantially exceeds the diameter of said face yarns, and in which the face warp has a cover factor whose value substantially exceeds the value for the cover factor of the face filling, said back filling yarns being equal in number per inch to the number of face filling yarns per inch.

6. A woven fabric of high water resistance, having an unnapped face material of a short float weave, said weave having warp yarn floats of up to four face filling yarns and face filling floats of up to eight face warp yarns, said face yarns being integrated with additional floated filling adapted to form a napped backing, said fabric comprising face warp and filling yarns, and back filling yarns floated under said woven face adapted to provide a pile-like back surface, in which the diameter of said back filling yarns substantially exceeds the diameter of said face yarns, and in which the face warp has a cover factor whose value substantially exceeds the value for the cover factor of the face filling, said face filling yarns being twice in number per inch to the number of back filling yarns per inch.

7. A woven fabric of high water resistance, having an unnapped face material of a short

float weave, said weave having warp yarn floats of up to four face filling yarns and face filling floats of up to eight face warp yarns, said face yarns being integrated with additional floated filling adapted to form a napped backing, said fabric comprising face warp yarns arranged in closely packed groups in an Oxford-type weave arrangement, face filling yarns, back filling yarns floated under said woven face adapted to provide a pile-like back surface, and additional binder warp yarns disposed beneath and concealed by groups of said face warp yarns and interlaced with said back and face filling yarns, the diameter of said back filling yarns substantially exceeding the diameter of said face yarns, and the face warp having a cover factor of a value substantially exceeding the value for the cover factor of the face filling.

8. A woven fabric of high water resistance, having an unnaped face material of a short float weave, said weave having warp yarn floats of up to four face filling yarns and face filling floats of up to eight face warp yarns, said face yarns being integrated with additional floated filling adapted to form a napped backing, said fabric comprising face warp yarns arranged in closely packed groups in an Oxford-type weave arrangement, face filling yarns, back filling yarns floated under said woven face adapted to provide a pile-like back surface, and additional binder warp yarns disposed beneath and concealed by groups of said face warp yarns and interlaced with said back and face filling yarns, said face filling yarns being equal in number per inch to the number of said back filling yarns per inch, the diameter of said back filling yarns substantially exceeding the diameter of said face yarns, and the face warp having a cover factor of a

10

15

25

30

35

value substantially exceeding the value for the cover factor of the face filling.

9. A water resistant fabric according to claim 4, wherein said face warp yarns and face filling yarns are members of the group consisting of cotton and spun synthetic staple yarns, and wherein said back filling yarns are members of the group consisting of wool and spun synthetic staple yarns.

10. A water resistant fabric according to claim 4, wherein said face warp and face filling yarns are cotton and wherein said back filling yarns are shrink resistant wool.

11. A water resistant fabric according to claim 4 wherein said back filling yarns have a float length of about .05 to about .2 inch.

12. A water resistant fabric according to claim 4, wherein said face warp yarns and face filling yarns are members of the group consisting of cotton and spun synthetic staple yarns, and wherein said back filling yarns are members of the group consisting of wool and spun synthetic staple yarns and have a float length of from about .05 to about .2 inch.

LOUIS LOVE.

## REFERENCES CITED

The following references are of record in the file of this patent:

## UNITED STATES PATENTS

| Number    | Name   | Date          |
|-----------|--------|---------------|
| 2,316,254 | Khoury | Apr. 13, 1943 |

## FOREIGN PATENTS

| Number | Country       | Date    |
|--------|---------------|---------|
| 3,267  | Great Britain | of 1905 |